

Patented Mar. 23, 1954

2,673,149

# UNITED STATES PATENT OFFICE

2,673,149

## QUATERNARY SALTS IN MIXED GRAIN PHOTOGRAPHIC EMULSIONS

Burt H. Carroll, Rochester, N. Y., assignor to Eastman Kodak Company, Rochester, N. Y., a corporation of New Jersey

No Drawing. Application October 17, 1951, Serial No. 251,833

6 Claims. (Cl. 95-2)

**1**  
This invention has to do with photography and particularly to the sensitizing of mixed grain emulsions.

The sensitization of mixed grain photographic emulsions has been described in Carroll and Hanson U. S. Patent 2,592,243. That application describes a method of overcoming the undesirable results of sensitizer diffusion. However, diffusion is seldom completely eliminated and the difficulties are greatest in those cases where the composition of the emulsions is different, since the affinity of the sensitizing dye for the silver halide grains varies with the silver halide used. In general, affinity is less for silver chloride than for silver bromide, so that there is the most difficulty when it is necessary to avoid diffusion of dye from an emulsion high in silver chloride to a bromoiodide emulsion, or a chlorobromide emulsion high in silver bromide. This situation is likely to occur in a single-layer, three-color emulsion where it is desirable to use high chloride emulsions for the red-sensitive and green-sensitive grains so that their blue sensitivity will be negligible compared to the blue-sensitive grains, or so that it can be eliminated entirely by use of a yellow printing filter.

It is, therefore, an object of the present invention to provide a novel method of sensitizing mixed grain photographic emulsions. A further object is to provide a method for preventing sensitizer diffusion in mixed grain emulsions. A still further object is to provide novel mixed grain photographic products. Other objects will appear from the following description of my invention.

These objects are accomplished by adsorbing quaternary salts on the surface of the silver halide grains of a mixed grain photographic emulsion.

My invention comprises in general the provision of a mixed grain photographic emulsion having two or more sets of silver halide grains sensitive to different spectral regions, in a hydrophylic carrier, one or more of the sets of grains having a quaternary salt adsorbed thereto.

The silver halide may be silver chloride, silver bromide, silver chlorobromide, silver bromoiodide, etc., in a carrier such as gelatin, polyvinyl alcohol, hydrolyzed cellulose esters or ethers, etc.

The quaternary salts which I may use are quaternary salts of compounds having the formula:



**2**  
where  $Z$  represents the atoms necessary to complete an azole ring, preferably an azole ring having a fused-on arylene nucleus, e. g., thiazole, benzothiazole, benzoxazole, benzoselenazole, naphthothiazole, etc., and  $n$  is an integer from 5 to 10. The quaternary salt may be a chloride, bromide, iodide, sulfate, *p*-toluenesulfonate, perchlorate, etc.

The quaternary salts which I prefer to use have the formula:



where  $n$  is an integer from 5 to 10 inclusive. Other anions may be present instead of  $-\text{ClO}_4$ , e. g. chloride, bromide, iodide, sulfate, *p*-toluenesulfonate, etc. The following are suitable compounds: Pentamethylene-bis-benzothiazolium perchlorate, heptamethylene-bis-benzothiazolium perchlorate, decamethylene-bis-benzothiazolium perchlorate. Other bis quaternary salts of antifoggants may be used, e. g. the bis quaternary salts of the thiazoles, naphthothiazoles, benzoxazoles, benzoselenazoles, and related heterocyclic nuclei, with or without substitution such as alkyl, aryl, alkoxy or halogen, disclosed in Brooker and Staud U. S. Patent 2,131,038.

The optical sensitizing dyes useful in my mixed grain emulsions embrace the following:

(1.) Carbocyanines derived from  $\beta$ -naphthothiazole substituted in the central position of the chain by alkyl or aryl groups (Brooker U. S. Patent 1,846,301).

These include

3,3'-dimethyl-9-ethyl-4,5,4',5'-dibenzthia-carbocyanine chloride.  
3,3'-dimethyl-9-phenyl-4,5,4',5'-dibenz-thiacarbocyanine bromide.  
3,3',9-triethyl-4,5,4',5'-dibenzthiacarbocyanine bromide.

45 Corresponding dyes from  $\beta$ -naphthothiazole nuclei substituted in the nucleus by halogen, alkyl or alkoxy may also be used and the alkyl groups on the 3-positions may be replaced by hydroxy-alkyl or carboxyalkyl and the aryl group in the 9-position may be substituted by alkyl, halogen, or alkoxy. These are red sensitizers.

(2.) Carbocyanines derived from substituted benzothiazole or benzoselenazole nuclei substituted in the central position of the chain by alkyl or aryl groups, for example, 3,3',9-triethyl-5,5'-

dichloroselenacarbocyanine bromide (made by the method of White U. S. Patent 1,990,681, using 5-chloro-2-methylbenzoselenazole instead of 2-methylbenzoselenazole). These are red sensitizers.

(3.) 3,3' - dimethyl - 8,10 - aryloxythiacarbocyanines and oxacarbocyanines (Brooker and White U. S. Patent 2,478,366).

These include

3,3' - dimethyl - 8,10 - m - toloxythiacarbocyanine bromide.

3,3' - dimethyl - 8,10 - m - toloxyoxacarbocyanine bromide.

These are red and green sensitizers, respectively.

(4.) Carbocyanines derived from 5-phenylbenzoxazole or 5-(p-tolyl)-benzoxazole, substituted in the central position of the chain by alkyl or aryl groups, for example, 3,3',9-triethyl-5,5'-di-p-toloxacarbocyanine bromide (see British Patent 496,116). These are green sensitizers.

(5.) Certain 2'-cyanines, for example, 1',3-diethyl - 5 - phenyl-6'-methoxy thia-2'-cyanine bromide (Van Zandt and Brooker U. S. application Serial No. 711,816, now Patent No. 2,515,913), and 1',3-diethyl-4,5-benz-6'-methylthia-2'-cyanine bromide (Brooker U. S. Patent 1,935,696). These are green sensitizers.

The optical sensitizing dyes are preferably used at a concentration of from 7 to 50 mg. of sensitizing dye per liter of silver halide emulsion containing about 0.25 gram mole of silver halide per liter of emulsion.

According to my invention, the silver halide emulsion is treated with the quaternary salt before or after optical sensitizing. In the case of the blue sensitive component of the mixture, no optical sensitizing dye is ordinarily used. With the red-sensitive and green-sensitive components of the mixture, the silver halide is optically sensitized to the desired spectral region and is then treated with the quaternary salt, although the quaternary salt may be omitted from these grains if used on the unsensitized blue-sensitive grains. The amount of quaternary salt may vary from about 20 to 400 milligrams per mole of silver halide. To form the mixed grain emulsion, silver halide emulsions sensitized to different spectral regions are mixed in approximately equal amounts or in amounts containing approximately equal quantities of silver.

The following example illustrates the formation of a mixed grain emulsion according to my invention:

To a blue-sensitive silver halide emulsion containing 98 mole-percent silver bromide and 2 mole-percent silver chloride there was added decamethylene-bis-benzothiazolium perchlorate in the proportion of 175 mg. per mole of silver halide and the emulsion was digested with it for 5 minutes at 50° C., then cooled to coating temperature of about 40° C.

A red-sensitive emulsion containing bromide equal to 20 mole-percent of the silver and chloride in excess of the remaining 80 mole-percent was sensitized with 3,3'-dimethyl-9-phenyl-4,5,4',5'-dibenzthiacarbocyanine chloride, 88 mg. per mole of silver halide, and digested 5 minutes at 50° C. with the dye. After cooling to 40° C., decamethylene-bis-benzothiazolium perchlorate, in the amount of 175 mg. per mole of silver halide was added.

To a green-sensitive emulsion of the same

silver halide composition as the red-sensitive emulsion, there was added 3,3',9-triethyl-5,5'-diphenyl oxacarbocyanine bromide in the amount of 88 mg. per mole of silver halide, the emulsion was digested 5 minutes at 50° C. and then cooled to 40° C. and decamethylene-bis-benzothiazolium perchlorate was added in the amount of 175 mg. per mole of silver halide.

The usual spreading agents and hardener were added to each of the emulsions and the emulsions were then mixed in amounts containing equal amounts of silver and immediately coated.

After drying, this coating was exposed to a color chart and processed as described in Example 4 of U. S. Patent 2,592,243 of Carroll and Hanson. There was no detectable diffusion of sensitizing dyes.

It will be understood that these examples are illustrative only and that modifications may be made in the method and material within the scope of the appended claims.

I claim:

1. A mixed grain photographic emulsion containing at least two sets of silver halide grains sensitive to different spectral regions, at least one of said sets of grains being sensitized with a cyanine sensitizing dye and at least one of said sets of grains having adsorbed thereto a quaternary salt of the structure:



where  $n$  is an integer from 5 to 10.

2. A mixed grain photographic emulsion containing at least two sets of silver halide grains sensitive to different primary colors, at least one of said sets of grains being sensitized with a cyanine sensitizing dye and at least one of said sets of grains having adsorbed thereto a quaternary salt of the structure:



3. A mixed grain photographic emulsion containing sets of silver halide grains sensitive respectively to the blue, green and red spectral regions, at least one of said sets of grains being sensitized with a cyanine sensitizing dye and at least said blue-sensitive grains having adsorbed thereto a quaternary salt of the structure:



4. A mixed grain photographic emulsion comprising a mixture of a blue-sensitive gelatino-silver halide emulsion, a cyanine-sensitized green-sensitive gelatino-silver chlorobromide emulsion, and a cyanine-sensitized red-sensitive gelatino silver-chlorobromide emulsion, said blue-sensitive emulsion having adsorbed to the silver halide grains a quaternary salt of the structure:



5. The method of preventing sensitization of silver halide grains by diffused optical sensitizer in a mixed grain photographic emulsion, which comprises treating at least one silver halide emulsion with a quaternary salt of the structure:



where  $n$  is an integer from 5 to 10, and mixing said emulsion with at least one other silver halide emulsion, each of said emulsions being sensitive to a different spectral region and at least one of said emulsions being sensitized with a cyanine optical sensitizing dye.

6. The method of preventing sensitization of

silver halide grains by diffused optical sensitizer in a mixed grain photographic emulsion, which comprises treating at least one silver halide emulsion with decamethylene-bis-benzothiazolium perchlorate, and mixing said emulsion with at least one other silver halide emulsion, each of said emulsions being sensitive to a different spectral region and at least one of said emulsions being sensitized with a cyanine optical sensitizing dye.

BURT H. CARROLL.

References Cited in the file of this patent

UNITED STATES PATENTS

15 Number Name Date  
2,288,226 Carroll et al. June 30, 1942